

Dec. 14, 1937.

S. E. SHEPPARD ET AL

2,101,877

PROCESS FOR PREPARING PHOTOGRAPHIC GELATIN

Filed Sept. 6, 1935

*Fig.1.*



*Fig.2.*



INVENTORS:

*Samuel E. Sheppard & James H. Hudson*

BY *Winton M. Perrine*

ATTORNEY.

## UNITED STATES PATENT OFFICE

2,101,877

## PROCESS FOR PREPARING PHOTOGRAPHIC GELATIN

Samuel E. Sheppard and James H. Hudson,  
Rochester, N. Y., assignors, by mesne assignments,  
to Eastman Kodak Company, Jersey  
City, N. J., a corporation of New Jersey

Application September 6, 1935, Serial No. 39,455

4 Claims. (Cl. 87—7)

This invention relates to a process of producing gelatin for photographic uses.

In the usual procedure for obtaining photographic gelatin from hides, the hides are first washed with water to remove dirt and foreign matter and are then soaked in saturated lime water which generally contains a considerable amount of free lime. This removes the hair, and this depilatory process is also accelerated by the formation of sulfides by inter-action of lime with young hair substances. The fats are next saponified and converted to lime soaps. After this the hide is subjected to a swelling in alkaline solution, whereby the soluble albumens diffuse out, together with other soluble substances which are photographically active and tend to cause fogging in the sensitive emulsions produced from the gelatin. This swelling in the alkaline bath for plumping may require from one to several months. The stock is then partially neutralized with an aqueous acid and the gelatin extracted by treating with water.

The gelatins produced in this way exhibit a general uniform type of colloid behavior. These properties are at a decided minimum at a hydrogen ion concentration of about 4.9. This minimum also corresponds to the iso-electric point of such gelatins. It has been found that although the duration of extraction, the concentration of the gelatin at the time of setting to a jelly, and other minor variations affect the colloid properties to some extent, these variations are, however, secondary and do not prevent gelatins obtained by alkaline treatment from exhibiting the same general type of colloid behavior.

We have discovered that if gelatin is obtained by a wholly acid treatment of hides, the resulting gelatin has colloid properties distinctly different from those of gelatin obtained by alkaline treatment of hides. The properties of this acid gelatin are such as make it particularly desirable for use as a photographic gelatine.

It is, therefore, an object of the present invention to provide a method for obtaining gelatin from hides by a completely acid process. It is a further object to provide a method for making a photographic gelatin having reduced swelling properties in alkaline solution and possessing other colloid properties different from those of gelatin obtained by alkaline treatment of hides.

In the accompanying drawing, Figure 1 is a graphic representation of the colloid properties of gelatin obtained by alkaline treatment of hides. Figure 2 is a graphic representation of the colloid

properties of gelatin obtained by our acid treatment of hides.

According to our improved method of obtaining photographic gelatin, the hides, such as calf-skin, are first washed to remove dirt or foreign matter and are chopped into pieces of approximately uniform size, for example, of about 8 to 10 square inches. These pieces are then soaked in an excess of dilute acetic acid. The concentration of this acid may vary from  $\frac{1}{2}$  to 2%, depending upon the age and condition of the stock. During treatment in the acid bath, the hide pieces are agitated from time to time to insure complete action by the acid. In about six or eight days the hair, still embedded in the exterior cuticle or epidermis, will loosen and may be removed from the hide by rubbing or agitation.

The partly swollen residual hide pieces are then left in the acid for a sufficient time for full plumping to take place. This action may be completed in a week, or it may require a somewhat longer time.

After plumping, the acid liquor is drained from the stock and the hide pieces are then neutralized to a pH of six to seven. This is carried out in the following manner: The hide pieces are placed in an aqueous solution and the solution adjusted to the desired pH by addition of an alkaline material. After the hide pieces have remained in this solution for an appreciable time, one of the pieces is removed and sliced through the middle to obtain an exposed section. The exposed section is coated with an indicator solution which indicates pH of the hide piece upon comparison of the color with a standard chart. If the hide piece shows that the center of the piece has not reached the pH of the solution, the soaking of the remaining pieces is continued until testing in this manner shows that the centers of the pieces have reached the desired degree of neutralization. Indicators which may be used to determine the pH of the hide pieces in this way are Brom Cresol green which indicates pH in the range of pH 3.8 to 5.6, Chlorphenol red which indicates pH in the range of pH 5.2 to 6.8, and Brom thymol blue which indicates pH in the range of pH 6 to 7.6. Color nuance may be estimated with these dyes with an accuracy of pH 2 to 4.

Extraction of the gelatin is then carried out in the usual way by treating with water at a temperature of 170 to 180° F. A large part of the fat remains in the hides with the residual elastin prior to extraction of the gelatin, but most of it

comes through in melted condition with the gelatin liquor and may be separated by skimming or centrifuging. The gelatin liquor is then filtered and may be vacuum-concentrated before chilling and drying.

The colloid properties of gelatin which are used to distinguish one gelatin from another are properties such as swelling in water, change of viscosity in aqueous solution, and precipitation from solution by alcohol. In the accompanying drawing these colloid properties are grouped together and represented by the letter F. The letter F therefore represents a composite of the units in which the various colloid properties are expressed. For example, the swelling in water is determined by the increase in weight when the gelatin is placed in water for an appreciable length of time. In this case the letter F would represent the weight of the gelatin when placed in water at the various units of pH. In a similar manner change in viscosity in aqueous solution is measured by the time required for the solution to pass through an orifice of definite size. The time required at various units of pH would, therefore, be represented by the letter F. The precipitation from solution in alcohol is measured as the amount precipitated from a solution of definite concentration upon addition of alcohol to the solution. The amount precipitated would, therefore, be represented by the letter F in the present case. The curves obtained on plotting each of these properties separately against the pH are found to show a similar general outline. If these properties are plotted against the pH of a gelatin solution, it is found that, for gelatin obtained by alkaline treatment of hides, there is a sharp minimum in the curve at pH 4.9. This is represented by the curve A in Figure 1. For gelatin obtained by acid treatment of hides according to our process, the colloid properties when plotted against pH do not show a sharp minimum at the pH 5 region, but the curve has a flat minimum region from pH 7 onward. This flattening of the curve may vary and may assume the form of nearly a straight line, as indicated at B" in Figure 2, or there may be less flattening of the curve, as indicated at B'.

We have described our process with particular reference to the use of acetic acid in treating the hides. However, we are not limited to the use of this acid, any weakly ionized acid other than acetic being adaptable to our process. The treatment of the hides with such acids is extremely mild and the hides are exposed to hydrolysis for a much shorter time than in alkaline treatment, and for this reason a very strong gelatin solution is obtained. We have referred to the treatment of calf skins by our process, but it is obvious that other hides might be treated in a similar manner.

It will be seen, by reference to the curve shown in Figure 2 of the drawing, that gelatins obtained according to our process exhibit less swelling in alkaline solution than gelatines obtained by alkaline treatment of hides. This is illustrated by the flattened portion of the curve shown in the region of pH 7 onward. This property is of particular advantage in making photographic emulsions for use where alkaline conditions of processing are to be employed. An example of this is in tropical development where it is usually necessary to use a highly alkaline solution and to employ anti-swelling compounds to prevent excessive swelling of the gelatin. The use of our gelatin obviates the necessity of using such anti-swelling compounds in the development of highly alkaline solutions. Numerous other advantages are also obtained by the use of our acid-extracted gelatin.

What we claim and desire to secure by Letters Patent of the United States is:

1. A process of preparing photographic gelatin having a minimum region of colloidal properties, such as swelling in water and change in viscosity in alkaline solution, at pH 7 and upward, which comprises steeping, unhairing, and plumping hides in about a  $\frac{1}{2}$  to 2% solution of the weakly ionized acid, neutralizing the hides to a pH of about 6 to 7, and extracting the gelatin from them in water solution.

2. A process of preparing photographic gelatin having a minimum region of colloidal properties, such as swelling in water and change in viscosity in alkaline solution, at pH 7 and upward, which comprises steeping, unhairing, and plumping hides in about a  $\frac{1}{2}$  to 2% solution of acetic acid, neutralizing the hides to a pH of about 6 to 7, and extracting the gelatin from them in water solution.

3. A process of preparing photographic gelatin having a minimum region of colloidal properties, such as swelling in water and change in viscosity in alkaline solution, at pH 7 and upward, which comprises steeping, unhairing, and plumping calfskin in a dilute solution of a weakly ionized acid, neutralizing the hides to a pH of about 6 to 7 and extracting the gelatin from them in water solution.

4. A process of preparing photographic gelatin having a minimum region of colloidal properties, such as swelling in water and change in viscosity in alkaline solution at pH 7 and upward, which comprises steeping, unhairing and plumping calfskin in about a  $\frac{1}{2}$  to 2% solution of acetic acid; neutralizing the calfskin to a pH of about 6 to 7 and extracting the gelatin from it in water solution.

SAMUEL E. SHEPPARD.  
JAMES H. HUDSON.